

## UNITED STATES PATENT OFFICE

ROBERT D. PIKE, OF OAKLAND, CALIFORNIA

## PROCESS FOR VOLATILIZING PHOSPHORUS AND POTASH AND FOR PRODUCING POTASH-BEARING PHOSPHORIC ACID

No Drawing.

Application filed November 14, 1927. Serial No. 233,325.

This invention relates to the production of a potash-bearing phosphoric acid and a method of producing the same, preferably from phosphate rock and Wyomingite rock.

5 In southeastern Idaho occur large quantities of phosphate rock, and in southwestern Wyoming, about two hundred miles distant occurs a large tonnage of a high-grade Leucite rock containing about eleven per cent. (11%) of  $K_2O$  and known as "Wyomingite". These materials can be cheaply assembled at one point, and my present invention has for its object to provide a cheap process for producing from these a potash-15 rich phosphoric acid by volatilization in a coke-fired blast furnace. Whereas my invention is particularly adapted to the treatment of Wyomingite and phosphate rock, it will be understood that it may be equally 20 well suited for use of other, similar materials.

It is a well-known fact that it is possible to volatilize potash and phosphorus from mixes of phosphate rock, a potash-bearing 25 silicate and coke, in the electric furnace. It has also been proposed (United States Patent Number 1,592,757), that a coke-fired blast furnace be used for this purpose, using a mixture of one part phosphate rock and 30 about two parts of Wyomingite, with coke; but it was found necessary, according to this patent, in order to volatilize the potash from such a highly siliceous mixture, to inject salt or calcium chlorid at the tuyères.

35 There are several important objections to the last-named procedure, some of which are:

1. The formation of hydrochloric acid 40 which passes over with the top gas from the furnace;

2. The relatively large amount of slag which is formed per unit of valuable plant food volatilized;

45 3. The highly siliceous nature of the slag,

rendering commercial operations of a blast furnace difficult, if not impossible; and

4. The difficulty of collecting a solid potassium phosphate in a Cottrell precipitator under the conditions existing, which would tend to make the salt sticky in the presence of a small excess of phosphoric acid, and, on the other hand, if the phosphoric acid were deficient there would be a tendency to precipitate potassium chlorid, whose presence is objectionable in a potassium phosphate which will usually be sold on a chlorine-free basis.

50 My invention consists in the substantially complete volatilization of phosphorus and potash from mixtures of phosphate rock and Wyomingite or similar materials in a coke-fired blast furnace with a basic fluid slag, and with the production of a fume which will yield after oxidation and humidification a potash-bearing phosphoric acid 55 which is liquid under the usual conditions of precipitation in a Cottrell precipitator.

60 The present process is preferably carried out in connection with my process for volatilizing phosphorus, concurrently filed, being Serial Number 233,323, in which a blast furnace is employed which uses a blast of air enriched with oxygen, and is based on my discovery that if I charge a mixture of 65 one part phosphate rock and seven-tenths to eight-tenths part Wyomingite into such a furnace, together with from seventy to eighty pounds of coke to every one hundred pounds of phosphate rock so charged, I can effect a substantially complete volatilization 70 of both the phosphorus and potash in the charge without the addition of any chemicals to promote volatilization of the latter.

75 As a result of such volatilization, the fume 80 which is collected in the Cottrell precipitator or by other suitable means contains from .2 to .3 pounds  $K_2O$  per pound  $P_2O_5$ , and is a liquid as collected, and will flow out of the collector or precipitator. The residual 85

gas is free from injurious corrosive substances, and may be employed as a fuel gas. I have found that if the ratio of  $K_2O$  to  $P_2O_5$  goes much over .3 to 1, the viscosity of the acid rapidly increases, so as to finally become unmanageable at ordinary temperatures of collection. The phosphoric acid collected by my process, containing as it does from .2 to .3 pounds  $K_2O$  per pound of  $P_2O_5$ , is very valuable for preparing fertilizer compounds, and my method of making it is so cheap as to constitute a revolution in the art of producing phosphoric acid.

I have found that for the successful carrying out of my process in the coke-fired blast furnace, the following general conditions have to be observed:

1. The conditions in the hearth and bosh of the furnace must be strongly reducing;
2. The charge should be so proportioned as to give in the slag after complete elimination of  $K_2O$  and  $P_2O_5$  an excess of molecules of bases over molecules of acids of from ten to thirty per cent. (considering alumina as an acid);
3. The temperature of the slag should be from  $1450^\circ$  to  $1500^\circ$  C.;
4. The slag should remain in the hearth of the furnace not less than two hours (and preferably over four hours), so as to give time for complete elimination of both the potash and phosphorus.

As a specific example of carrying out my process, I charge a blast furnace with one part of phosphate rock and with eight-tenths parts of Wyomingite and .7 parts coke, giving a slag of about the following analysis:

|           | Per cent |
|-----------|----------|
| $SiO_2$   | 39.7     |
| $Al_2O_3$ | 11.9     |
| $CaO$     | 43.0     |
| $MgO$     | 5.4      |

The furnace is blown with an oxygenated blast at  $650^\circ$  C. containing 30% of oxygen by weight. The slag is flushed every three to six hours. The eliminations of phosphoric acid and potash are both above 85%, or substantially complete, and the ratio of  $K_2O$  to  $P_2O_5$  in the acid which is collected from the top gas is about (after oxidation and humidification), .29 to 1., which insures a good fluidity of the acid at the temperature of collection. It will be understood that the top gases as they issue from the top of the furnace, contain fumes of  $K_2O$  and  $P_2O_5$  and of phosphorus. The latter has to be burned to  $P_2O_5$  in any suitable manner by the admission of air. The air so admitted to burn the phosphorus will usually contain enough moisture for the formation of ortho phosphoric acid with the  $P_2O_5$  present; but if the air happens to be so dry as to be deficient in moisture for this purpose, the deficiency must be made up by introduc-

ing moisture into the gases before they enter the precipitator.

It will be understood that many of the details concerning proportions, temperatures, etc., are subject to considerable variation without departing from the spirit of my invention, as disclosed in the appended claims.

Although I have specified the use of Wyomingite, it will be obvious that any potash-bearing silicate may be employed, and that if necessary the composition of the slag can be controlled by addition of other fluxing materials, as, for example, lime stone or dolomite.

Having thus described my invention, what I claim and desire to secure by Letters Patent is:

1. The process for the substantially complete volatilization of phosphorus and potash from phosphate rock and Wyomingite, which consists in charging into a coke-fired blast furnace one part of phosphate rock with not more than eight-tenths part of Wyomingite, together with the necessary amount of coke for furnishing heat and a strongly reducing condition in the hearth and bosh of the furnace, flushing the slag from the furnace after a sufficient time of residence to insure the substantially complete volatilization of phosphorus and potash, adding air to the furnace top gases to oxidize all the phosphorus they contain to  $P_2O_5$ , and sufficient moisture to convert  $P_2O_5$  to ortho phosphoric acid, and collecting the phosphoric acid and potash.

2. The process of extracting potassium and phosphorus from potassium-bearing and phosphorus-bearing rocks, which consists in volatilizing the potassium and the phosphorus compounds by smelting the rocks under reducing conditions in a coke fired blast furnace, the charge being so proportioned that the slag contains an excess of basic molecules over acid molecules, treating the gases produced by the smelting operation to cause the formation of an acid compound of phosphorus and potassium, and thereafter recovering such compound from the gases in liquid form.

3. The process of extracting potassium and phosphorus from potassium-bearing and phosphorus-bearing rocks, which consists in volatilizing the potassium and the phosphorus compounds by smelting the rocks under reducing conditions in a coke fired blast furnace, the charge being so proportioned that the slag contains an excess of basic molecules over acid molecules, oxidizing and humidifying the gases to form ortho phosphoric acid and potassium phosphate, and simultaneously collecting these compounds.

4. The process for the substantially complete volatilization of phosphorus and potash from phosphate rock and a potash-bear-

- ing silicate, which consists in charging into a coke-fired blast furnace one part of phosphate rock with not more than eight-tenths part of potash-bearing silicate, together with the necessary amount of coke for furnishing heat and a strongly reducing condition in the hearth and bosh of the furnace, flushing the slag from the furnace after a sufficient time of residence to insure the substantially complete volatilization of phosphorus and potash, and recovering said phosphorus and potash. 5
5. The process for the substantially complete volatilization of phosphorus and potash from phosphate rock and Wyomingite, which consists in charging into a blast furnace fired with solid carbonaceous fuel, one part of phosphate rock with not more than eight-tenths part of Wyomingite, together with the necessary amount of solid carbonaceous fuel, for furnishing heat and a strongly reducing condition in the hearth and bosh of the furnace, flushing the slag from the furnace after a sufficient time of residence to insure the substantially complete volatilization of phosphorus and potash, adding air to the furnace top gases to oxidize all the phosphorus they contain to  $P_2O_5$  and sufficient moisture to convert  $P_2O_5$  to ortho phosphoric acid, and collecting the phosphoric acid and potash. 10
6. The process of extracting potassium and phosphorus from potassium-bearing and phosphorus-bearing rocks, which consists in volatilizing the potassium and the phosphorus compounds by smelting the rocks under reducing conditions in a blast furnace fired with solid carbonaceous fuel, the charge being so proportioned that the slag contains an excess of basic molecules over acid molecules, treating the gases produced by the smelting operation to cause the formation of an acid compound of phosphorus and potassium, and thereafter recovering such compound from the gases in liquid form. 15
7. The process of extracting potassium and phosphorus from potassium-bearing and phosphorus-bearing rocks, which consists in volatilizing the potassium and the phosphorus compounds by smelting the rocks under reducing conditions in a blast furnace fired with solid carbonaceous fuel, the charge being so proportioned that the slag contains an excess of basic molecules over acid molecules, oxidizing and humidifying the gases to form ortho phosphoric acid and potassium phosphate, and simultaneously collecting these compounds. 20
8. The process for the substantially complete volatilization of phosphorus and potash from phosphate rock, and a potash-bearing silicate, which consists in charging into a blast furnace fired with solid carbonaceous fuels one part of phosphate rock with not more than eight-tenths part of potash-bearing silicate, together with the necessary amount of solid carbonaceous fuel for furnishing heat and a strongly reducing condition in the hearth and bosh of the furnace, flushing the slag from the furnace after a sufficient time of residence to insure the substantially complete volatilization of phosphorus and potash, and recovering said phosphorus and potash. 25
- ROBERT D. PIKE. 30
- 80
- 85
- 90
- 95
- 100
- 105
- 110
- 115
- 120
- 125
- 130